

March 10, 1925.

1,529,046

E. E. WINKLEY

HEEL AND METHOD OF MAKING THE SAME

Original Filed Jan. 25, 1918



*Fig. 1.*



*Fig. 2.*



*Fig. 3.*



*Fig. 4.*



*Fig. 5.*



*Fig. 6.*



*Fig. 7.*



*Fig. 8.*

*Witness,*

*Poorill C. Hatch.*

*Inventor:*

*Erastus E. Winkley  
by his attorney  
Harrington, Tracy & Hildreth*

Patented Mar. 10, 1925.

1,529,046

# UNITED STATES PATENT OFFICE.

ERASTUS E. WINKLEY, OF LYNN, MASSACHUSETTS, ASSIGNOR TO UNITED SHOE MACHINERY CORPORATION, OF PATERSON, NEW JERSEY, A CORPORATION OF NEW JERSEY.

## HEEL AND METHOD OF MAKING THE SAME.

Application filed January 25, 1918, Serial No. 213,682. Renewed June 20, 1923.

To all whom it may concern:

Be it known that I, ERASTUS E. WINKLEY, a citizen of the United States, residing at Lynn, in the county of Essex and state of Massachusetts, have invented certain new and useful Improvements in Heels and Methods of Making the Same; and I do hereby declare the following to be a full, clear, and exact description of the invention, such as will enable others skilled in the art to which it appertains to make and use the same.

This invention relates to the preparation of heels of leather, leatherboard or analogous leather or paper compositions or combinations thereof, and includes the method of making off the shoe, compressed and definitely shaped heels, and the novel heel produced by following some or all of the steps hereinafter described as desirable in practising the method.

One of the objects of the present invention is to improve and develop the method of making heels set forth in a co-pending application, Serial No. 213,681, filed of even date herewith by the present inventor, in which claims will be found dominating broadly the method herein disclosed and certain novel features of the resulting product.

Another object of this invention is to provide a simple and expeditious method of making compressed heels of not only final size and shape but also of making complete unitary and entirely finished heels "off the shoe," that is, heels that are built and ultimately finished before attachment to the shoe.

Another object is to provide a practical method of making "off the shoe" a complete unitary heel that shall be adapted for use in conjunction with short-soles and which may embody at least a base-lift of leatherboard, or other of the cheaper grades of heel-stock, that is acted upon in such a manner that the lateral surface of the base-lift or heel, to an appreciable depth, undergoes a change, and its characteristics are so improved and modified that it is particularly adapted to take a clean-shaped, smooth and durable randing cut, a distinct and permanent beading or key-wheel marking, and a finish or polish that compare favorably with that of all-leather heels or heels having base-lifts of leather.

In practising the method of the present invention in its preferred form, rough heel-piles of the desired lift material are built up and finally nailed together, after which a suitable top lift is attached and slugged. The resulting heel-pile is then trimmed, shaved or otherwise formed into definite shape. This heel is then moulded in a compressor to substantially final size and form, whereby the heel is consolidated and compacted around the nails and slugs, the slugs are forced slightly below the surface of the top-lift, and the lateral surface of the heel is materially improved, and adapted for the subsequent finishing operations. The lateral surface of the heel, especially if made from the cheaper heel-stock materials, is further modified and improved by being filled with a suitable sizing material before compressing. Practice has determined that a glutinous material is well adapted as a sizing agent, although the invention is not so restricted as any material for producing the desired results may be employed.

The step of filling the lateral surface of the heel, or at least of the base-lift after the trimming or shaping operation and before compression is especially important in making complete unitary heels that are to be finally finished before attachment to the shoe, and which are employed in connection with short soles, for the reason that the resulting lateral surface is such that it may be readily worked upon with tools such as are used to cut the usual randing and to produce the beading or key-wheel marking. Without this treatment, the use of leatherboard for base-lifts of heels is impractical, since the composition is such that in cutting the randing, the surface is liable to flake off or tear out, thus impairing the smoothness of the subsequent finish and spoiling the heels. The sizing, however, penetrates into the pores that are opened up by the previous trimming operation, and after compression, a firm, hard and smooth outer lateral surface of appreciable depth is formed, in which a clean-cut, durable randing, and sharp and permanent key-wheel marking or beading may be produced.

The present method may be practised in connection with heel stock material of any character, but is particularly adapted to be employed in the manufacture of heels composed of superposed lifts of leatherboard.

or other of the cheaper and analogous compositions of leather or paper. The term "leatherboard," therefore, is used in a generic sense to include any suitable heel-stock material.

The term "lift" is also used in an inclusive sense to define any blank or layer of material that is adapted for use in the formation of heel-piles from which heels are ultimately produced, irrespective of the particular shape of the blanks or the nature of the material of which they are composed.

From the foregoing it will be understood that the invention comprises both the method 15 of making heels, hereinafter described in detail, and the heel which results from practising the method, as defined by the appended claims.

The particular steps employed in preparing 20 the novel article of manufacture and their preferred sequence, as well as the preferred form of the article, will now be explained in connection with the accompanying drawings, in which Figure 1 is a perspective view of a rough heel-pile built up of superposed lifts of polygonal form; Fig. 2 is a perspective view of the heel-pile shown in Fig. 1, which has been permanently nailed together, the ends of the nails protruding 25 slightly from the tread end of the heel-pile; Fig. 3 is a perspective view of the heel-pile with a top-lift attached. Fig. 4 is a similar view of the heel-pile shown in Fig. 3 after slugs have been driven into the top-lift; Fig. 5 is a view in perspective of a preliminarily shaped heel of definite form that has 30 been trimmed from the heel-pile illustrated in Fig. 4; Fig. 6 is a similar view of a shaped heel in position in a mould and about to be compressed to final size and form, the lateral 35 surface of which may have been previously filled with a sizing material; Fig. 7 is a perspective view of a heel compressed to final size and form with the randing cut upon the upper edge of the base lift, and Fig. 8 is a 40 similar view of a completely finished heel that has been subjected to the necessary or desirable finishing operations, after which the beading or key-wheel marking has been impressed and the heel thus made ready for 45 subsequent attachment to a shoe having a short outsole.

In accordance with the preferred method of practicing the invention, a rough heel-pile 50 (Fig. 1) of superposed lifts of leatherboard is built up and temporarily secured together in any well-known manner. As shown, the heel-pile is formed of polygonal lifts, although lifts of any shape may, 55 of course, be employed, and it embodies a leatherboard base-lift 12 that is somewhat shorter than the other lifts and is indented slightly from the breast end of the heel-pile.

The component lifts of this rough heel-pile 60 are then permanently and finally se-

cured together by means of nails 14 that are positioned so as to protrude slightly from the tread end of the heel, as shown in Fig. 2. A top-lift 16 is then spanked on or attached in a well-known manner (Fig. 70 3), and subsequently a row of slugs 18 (Fig. 4) is driven into the top-lift in accordance with customary practice. Obviously, the use of slugs is optional and may be omitted if desired. Furthermore, they may 75 be positioned in the top-lift before it is attached to the heel-pile.

The preliminarily formed rough heel-pile, as illustrated in Fig. 4, is then trimmed or formed in any suitable manner to a definite 80 and regular shape that corresponds to the shape of the heel when finished, but which is slightly larger in dimensions, in order that it may be subsequently consolidated and compressed in a suitable mould. The trimming operation is preferably performed in a machine similar to that set forth in Letters Patent No. 1,102,310 granted July 7, 1914, to the present applicant, by means of which the heel-pile is shaved or cut off to a 90 definite shape by a series of rapidly rotating knives. Any suitable means for definitely shaping the rough heel-pile, however, may be employed. Fig. 5 represents a shaped heel that has been trimmed or cut from the 95 rough heel-pile illustrated in Fig. 4.

If deemed desirable the lateral surface of the shaped heel, or at least of the base-lift thereof, is then filled with a suitable sizing material, and at this stage of the process, 100 the shaped heel is particularly adapted to receive the sizing, since its surface is somewhat roughened and the pores opened up as a result of the previous trimming or shaving operation. The sizing material, 105 therefore, penetrates the surface of the heel to an appreciable extent and also serves to raise or turn out the exposed fibres.

Assuming that the whole or a portion of the lateral surface of the shaped heel has 110 been treated in the general manner referred to, the sizing is preferably permitted to dry to a greater or less extent, after which the shaped and sized heel is placed into a suitable mould or compressor, as illustrated in 115 Fig. 6, preferably such as set forth in Letters Patent No. 1,334,478, issued March 23, 1920, to the present applicant. The heel is then moulded or compressed under heavy 120 pressure to its final size and form, during which operation the heel as a whole is condensed and consolidated, while the outer fibres that have been raised by the sizing material are turned in and forced into the lateral surface of the heel, which is thus compacted and rendered particularly hard and smooth.

The sizing treatment and subsequent compression results in effecting a change in the 125 characteristics and properties of the lateral 130

surface of the heel, which render it especially adapted to take the subsequent finishing operations and which produce in the leatherboard base-lift a lateral surface having properties that permit the cutting of a smooth and clean-cut randing and a distinct and permanent key-wheel marking or beading.

The compressing operation on a definitely shaped heel is especially effective in producing a hard and consolidated lateral surface on the heel. It also serves to compact the body of the heel around the nails and slugs, while forcing the exposed ends of the slugs flush with the tread surface of the top-lift, by reason of which they become slightly depressed below said surface upon the slight expansion of the heel-stock material after removal from the compressor mould.

Subsequent to the compressing operation, illustrated in Fig. 6, a randing 20 (Fig. 7) is cut around the upper edge of the base-lift 12 in any well-known manner, and as a result of the previous treatment of the heel, this cutting operation is facilitated and a clean-cut and smooth randing is insured.

The heel is then subjected to the usual finishing operations, such as scouring, blacking, burnishing, breasting, etc., as a result of which the heel is ultimately finished and polished, after which the key-wheel marking or beading is impressed upon the edge of the base-lift. Thus, a completely finished unitary heel is produced "off the shoe," which is ready for application and attachment to a shoe having a short outsole.

By reason of the fact that the heel is compressed to final size and shape, it requires no further trimming or alteration, and the improved and beneficial qualities of the lateral surface of the heel are retained and contribute to a complete heel of superior finish and durability. Moreover, inasmuch as the heel is compressed to final and definite shape and size, only light scouring operations are necessary, which are insufficient to remove and cut beneath the improved and modified surface of the heel, so that the benefits of the improved qualities are not sacrificed by removal during the finishing operations. The finishing of the tread surface of the top-lift is particularly facilitated by reason of slugging the top-lift before compression, inasmuch as the ends of the slugs are slightly depressed beneath the surface of the compressed heel, so that only a slight amount of scouring of the slugs and top-lift surface is required.

In the above process, the step of trimming or shaping the rough heel-pile is of special importance, for the reason that the shaped heel is adapted to fit closely within the mould of the compressor throughout its entire surface, whereby the pressure to

which the heel is subjected is uniformly distributed, thus resulting in a more uniformly consolidated product. Moreover, the trimming operation roughens the lateral surface and opens the pores of the heel, so that the penetration of the sizing material, when used, is increased and rendered particularly effective.

The sizing or filling step is also advantageous in that it contributes to the improved and modified characteristics and properties of the lateral heel surface, which materially aid in finishing the heel and which are particularly important in unitary heels of leatherboard that are completely finished "off the shoe," the base-lift of which must be randed and impressed with key-wheel markings.

In describing the trimming of the heel to definite shape and its compression to final size and form, the specification obviously refers to the lateral surface of the heel, inasmuch as the heel is subsequently breasted during the customary finishing operation.

Although the method of preparing the heel has been set forth as including a predetermined sequence of steps, those skilled in the art will readily understand that omissions and variations of some of the steps may be made within the spirit and scope of the invention, and therefore it is desired that only such limitations shall be imposed as are indicated in the appended claims.

Having thus described the novel features of the heel of the present invention and the preferred method by which it may be prepared, that which is claimed as new, is:-

1. The method of making heels that are finished before attachment to the shoe, which comprises building a rough heel-pile of superposed lifts, nailing together the component lifts thereof, attaching a top-lift thereto, trimming the resulting products to definite shape, compressing the shaped heel to final size and form, and subsequently finishing the heel ready for application to a shoe.

2. The method of making heels which includes building a rough heel-pile of superposed lifts, nailing together the component lifts thereof, attaching a top-lift thereto, trimming the resulting product to definite shape, and moulding the shaped heel under heavy pressure.

3. The method of making heels which includes building a rough heel-pile of superposed lifts, nailing together the component lifts thereof, slugging and attaching a top-lift, trimming the resulting product to definite shape, and moulding the shaped heel under heavy pressure.

4. The method of making heels which includes building a rough heel-pile of superposed lifts, attaching a top-lift thereto,

trimming the resulting product to definite shape, and compressing the shaped heel.

5. The method of making heels which includes building a rough heel-pile of superposed lifts, slugging and attaching a top-lift, trimming the resulting product to definite shape, and compressing the shaped heel.

6. The method of making heels that are finished before attachment to the shoe, 10 which comprises building a rough heel-pile of superposed lifts, attaching a top-lift thereto, trimming the resulting product to definite shape, compressing the shaped heel to final size and form, and finishing the heel 15 ready for application to a shoe.

7. The method of making heels that are finished before attachment to the shoe, which comprises building a rough heel-pile 20 of superposed lifts, attaching a top-lift thereto, trimming the resulting product to definite shape, filling the surface of the shaped heel with sizing material, compressing the shaped and sized heel to final size, cutting the randing upon the compressed heel, and finishing the heel ready for application to a shoe.

8. The method of making heels that are finished before attachment to the shoe, which comprises building a rough heel-pile 30 of superposed lifts with a leather top-lift and a base-lift of leatherboard, trimming the heel-pile to definite shape, filling the surface of at least the base-lift of the shaped heel with sizing material, compressing the 35 shaped and sized heel to final size, cutting the randing in said leatherboard base-lift, and finishing the heel ready for application to a shoe.

9. The method of making heels which includes building a rough heel-pile of superposed lifts, nailing together the component lifts thereof, attaching a top-lift, trimming the heel-pile to definite shape, and compressing the heel under heavy pressure.

45 10. The method of making heels which comprises building a heel-pile of superposed lifts including a top-lift, slugging the top-lift, and then moulding or compressing the heel.

50 11. The steps in the method of making heels of superposed lifts which include slugging the top-lift and then compressing the heel with the top-lift in place.

55 12. The steps in the method of making heels of superposed lifts which include finally nailing together the component lifts and then compressing the heel into form.

60 13. The steps in the method of making heels of superposed lifts to be subsequently attached to a shoe which include attaching a top-lift to a rough heel-pile, trimming the heel-pile and top-lift to definite shape, and compressing the heel by heavy pressure applied directly to all the exterior surfaces 65 thereof.

14. The method of making heels for subsequent attachment to a shoe which comprises building a heel of superposed lifts including a leatherboard base-lift, filling the lateral surface of at least the base-lift of 70 the heel with sizing material, compressing the heel to final size, and cutting the randing in said leatherboard base-lift.

15. The steps in the method of making finished heels of superposed lifts, which include cutting the randing on the base-lift of 75 the heel, and then finishing the heel for subsequent attachment to the shoe.

16. A compressed and finally finished heel ready for attachment to a shoe, comprising 80 a plurality of superposed lifts, including a base-lift of leatherboard.

17. A compressed and finally finished heel ready for attachment to a shoe, comprising 85 a plurality of superposed lifts of leatherboard, the base-lift being indented from the breast edge and having a smooth, hard and compact surface of appreciable depth.

18. A compressed and finally finished heel ready for attachment to a shoe, comprising 90 a leatherboard base-lift, a leather top-lift and intermediate lifts all in superposed relation, the lateral surface of the base-lift being sized before compression, thereby rendering it smooth, hard and compact. 95

19. A compressed and finally finished heel ready for attachment to a shoe, comprising 100 a plurality of superposed lifts, including a sized and condensed leatherboard base-lift provided with a randing.

20. The method of making heels that are finished off the shoe which comprises building a rough heel-pile of superposed lifts, trimming the rough heel-pile to definite 105 shape, moulding the shaped heel under heavy pressure to its final size and form, and then finishing the heel ready for attachment to the shoe.

21. The method of making heels that are 110 finished before attachment to the shoe which comprises building a rough heel-pile of superposed lifts, trimming the heel-pile to definite shape, filling the lateral surface with sizing, compressing the shaped and sized heel to final size and form, and finishing the heel ready for application to a shoe. 115

22. The method of making heels which comprises building a heel-pile of superposed lifts, trimming the heel-pile to definite 120 shape, compressing the shaped heel to final size and form, and finishing the heel prior to attaching it to a shoe.

23. The method of making compressed heels of superposed lifts which comprises 125 nailing together the component lifts of a heel-pile, attaching a top-lift thereto, and subsequently moulding the resulting product to final size and form under heavy pressure. 130

24. The method of making compressed heels of superposed lifts which comprises nailing together the component lifts of a heel-pile, attaching a top-lift thereto, slugging the top-lift, and moulding the resulting product under heavy pressure. 50
25. A heel of superposed lifts, compressed to final size and form and completely finished for final attachment to a shoe. 55
- 10 26. A heel of superposed lifts, embodying a base-lift of leatherboard, compressed to final size and form, the base lift having a smooth, hard and compact lateral surface and the heel being completely finished and ready for final attachment to a shoe. 60
- 15 27. A compressed and finally finished heel ready for attachment to a shoe, comprising a plurality of superposed lifts, including a sized and condensed leatherboard base-lift. 65
- 20 28. A leatherboard heel, ready for attachment to a shoe, having its lateral surface sized, compressed to final form and finished. 70
- 25 29. A compressed heel including a top lift provided with slugs before compression. 75
- 30 30. The method of making heels which comprises building a heel of superposed lifts and of final size and form, finishing the lateral surface of said heel while off the shoe, 80 and subsequently attaching the finished heel to the shoe. 85
- 35 31. The method of building heels that are finished before attachment to the shoe which comprises building a heel-pile of superposed lifts, sizing the lateral surface of the heel-pile, compressing the sized heel-pile to final size and form, and then finishing the heel ready for attachment to the shoe. 90
- 40 32. The method of making heels to be subsequently attached to a shoe which includes building a heel-pile of superposed lifts including a top-lift, securing the component lifts of the heel-pile together, trimming the heel-pile to definite shape, and compressing the shaped heel-pile into a heel of final size and form. 95
- 45 33. The method of making heels for subsequent attachment to a shoe which comprises building a heel-pile of superposed lifts including a top-lift, sizing the lateral surface of the heel, and compressing the heel to final size and form. 50
34. The method of making heels for subsequent attachment to a shoe which comprises building a heel-pile of superposed lifts, filling the lateral surface of the heel with sizing material, compressing the sized heel to final size and form and finishing the heel ready for application to a shoe. 55
35. The method of making heels which includes forming a rough heel of superposed lifts including a top lift, trimming said heel to a definite shape, and compressing the heel, said trimming and compressing operations being performed while the heel is off the shoe. 60
36. The method of making heels which includes forming a rough heel of superposed lifts, nailing said lifts together leaving protruding nail ends, attaching a top lift to said protruding nail ends, trimming the resultant product to a definite shape, and compressing the shaped heel while off the shoe. 70
37. The steps in the method of making heels of superposed lifts which includes slugging and attaching a top lift to a rough heel pile, trimming the resultant product to a definite shape, and compressing the resultant heel to final size and form by heavy pressure applied directly to all the exterior surfaces thereof. 75
38. The method of making heels which includes forming a rough heel of superposed lifts all of similar contour, attaching said lifts together with a top lift at one end and a base lift indented from the breast edge at the other end, trimming said heel to a definite shape, and compressing the trimmed heel. 85
39. The method of making heels that are finished before attachment to the shoe which comprises trimming a rough heel to definite shape, filling the lateral surface with sizing, compressing the shaped and sized heel to final size and form, and finishing the heel ready for application to a shoe. 90

ERASTUS E. WINKLEY.